

Patented Aug. 8, 1933

1,921,363

# UNITED STATES PATENT OFFICE

1,921,363

## PROCESS FOR TREATING FIBERS

Georges Lefranc, Paris, France

No Drawing. Original application February 21, 1930, Serial No. 430,461, and in France January 11, 1930. Divided and this application July 11, 1931. Serial No. 550,292

3 Claims. (Cl. 91—68)

It is known that for sizing textile fibers emulsions of fatty or resinous substances are usually employed. The most usual emulsifying agents are sulphuricinoleates, or in most recent practice, other substances which like those above 5 specified, are derived from the sulphonic acids group.

For sizing fibers of animal origin these emulsions do not present any disadvantage but this is not the case when vegetable fibers are thus 10 treated. In fact cotton and its products such as artificial silk may indeed be injured or destroyed by such agents owing to hydrolytic action.

The attack may be so rapid, under favorable 15 temperatures or other conditions that, for example, it is not possible to export to tropical countries artificial silks sized by these processes, since the threads are found to be completely destroyed on arrival at their destination.

An example is hereinafter given which shows 20 to what degree the resistance and tensile strength of vegetable fiber is changed by the action of these agents.

A specimen A of viscose silk has been treated 25 with a size of ordinary composition. A specimen B of the same quality has been subjected to similar treatment but without the use of Turkey red oil.

The samples and a standard thread after being 30 kept for three weeks at a temperature of 50° C. showed the following resistances:

|                             | Resistance          |                   |
|-----------------------------|---------------------|-------------------|
|                             | In moist atmosphere | In dry atmosphere |
| 35                          |                     |                   |
| Standard sample not treated | 1.095               | 1.025             |
| Sample A                    | 0.510               | 0.570             |
| 40 Sample B                 | 1.095               | 1.045             |

In a like experiment, commercial samples of sized artificial silk have been found to lose up to 80% of their resistance.

45 The object of this invention is to obviate the employment, for sizing textile fibers and more particularly fibers of vegetable origin, of any substance liable to attack these fibers, including artificial silk, with a view to enabling the sized fibers to be exported to and used in tropical countries.

In particular the invention absolutely avoids 50 the use of sulphuricinoleates and other sulphonated compounds as emulsifying agents for the preparation of emulsions to be employed as sizes.

According to this invention emulsions of oils, 55 fats, resin or mixtures of the substances in a dispersion of casein, gelatin or shellac or a mixture of these substances are employed for this treatment. As dispersion agents alkaline borates

are employed. In order to obtain a neutral sodium or ammonium borate it is necessary to add to borax some soda lye or alkali (ammonia).

To the emulsion thus obtained, there is added, according to requirements, a soluble silicate so as to set up a reaction with the borate. By reason of the presence of protective colloids in the emulsion, the reaction product forms a colloids solution changed by desiccation to a gel which is irreversible in water at normal atmospheric temperatures. The granules of this gel present in addition an electrification of the surface of the same sign. By reason of this superficial ionic charge the fibers repel one another during drying and in this way sticking together of the fibers is avoided without detriment to the sizing.

The casein provides the strongest sizes. Borax may advantageously be used as the dispersion agent for avoiding adhesion of the threads. Casein swollen by steeping for several hours in water is therefore added to the borax solution. After a time (not exceeding two hours) the dispersion will have been completed. This solution is added gradually to fatty or resinous substances with regular agitation so as to obtain a thick homogeneous mass readily emulsifiable in an excess of water. The preservation of the flexibility brilliance and color of the fiber depends on the choice of the substances emulsified. Gum mastic dissolved in castor oil gives excellent results from this point of view. The sizes tend to become rather sticky or tacky in the neighborhood of 40° C. but this objection is easily overcome by substituting a vegetable fat such as palm oil in place of part of the castor oil. After standing for two hours a dilute solution of silicate of soda is added and the mixture is diluted with water and filtered twice through a filter of fine silk.

The emulsions thus prepared according to the invention disclosed in my co-pending application Serial No. 430,461, are employed for sizing fibers from different sources, either in a single bath, or by passing the fibers from the sizing bath through a deglutinating bath particularly when very fine fibers are being treated.

In this case the second bath can be of low concentration and the time of treatment of short duration.

In the composition of the deglutinating bath no substance is employed which might detrimentally affect the resistance of the fibers either directly or by hydrolysis which can easily be set up in hot or humid climates.

The deglutinating baths employed in carrying out the process are composed of formates, acetates and sulphocyanides of metals such as calcium, zinc, aluminium or lead.

By way of example and not by way of limitation the composition is hereinafter given of some emulsions complying with the characteristic above specified.

## Example 1

|                                         | grammes |
|-----------------------------------------|---------|
| Palm oil                                | 50      |
| Casein                                  | 10      |
| 5 Alkali (ammonia)                      | 25      |
| Distilled water                         | 100     |
| Borax                                   | 5       |
| Commercial solution of silicate of soda | 20      |

10 This size gives the fiber a mat appearance. The weight is increased 10%.

## Example 2

|                 | grammes  |
|-----------------|----------|
| 15 { Colophony  | 10       |
| { Cocoa-nut oil | 25       |
| { Casein        | 3        |
| { Soda lye      | 4        |
| Distilled water | 1,000    |
| 20 Borax        | 1        |
|                 | c. c. s. |

Commercial solution of silicate of soda 20

This gives a more brilliant sizing than Example 1 and increases the weight 10%.

25 The hanks are steeped in the bath which is stirred either by hand or mechanically during from one to three hours. After complete draining the hanks pass to a second bath of one of the three compositions as follows.

## 30 Example 3

|                  | grammes |
|------------------|---------|
| Aluminum acetate | 1       |
| Acetate of lime  | 1       |
| 35 Acetic acid   | 1       |
| Distilled water  | 100     |

## Example 4

|                           | grammes |
|---------------------------|---------|
| 40 Aluminum sulphocyanide | 10      |
| Acetic acid               | 1       |
| Distilled water           | 100     |

## Example 5

|                 | grammes |
|-----------------|---------|
| 45 Lead acetate | 5       |
| Acetic acid     | 1       |
| Distilled water | 100     |

The fiber is left in the second bath for a period of from half an hour to one hour and then dried.

50 The fibers are well sized and can be readily wound in skeins. They are resistant to the effects of high temperatures.

## Example 6

|                                           | grammes |
|-------------------------------------------|---------|
| 55 { Gum inastic                          | 24      |
| { Castor oil                              | 12      |
| { Palm oil                                | 12      |
| { Borax                                   | 6       |
| 60 { Distilled water                      | 200     |
| { Casein                                  | 8       |
| Distilled water                           | 100     |
| { Commercial solution of silicate of soda | 5       |
| Distilled water                           | 500     |

65 The soaked casein is added to the solution of borax and after standing for from two to four hours, the mixture is added little by little to the solution of the gum in the oils, the two ingredients of the emulsion being brought to the same temperature. After standing for two hours the dilute solution of silicate of soda is added the mixture is

made up with water to 2,000 grammes and is filtered twice through a filter of fine silk.

This sizing product (Example 6) can be employed without a second bath particularly for sizing threads of good quality. After draining the threads are dried at a temperature of about 60° C. The threads fall apart during this operation. The deglutination of the threads can be completely effected, before drying, by immersion for 5 to 30 minutes in a bath of one of the solutions as given in Examples 3, 4, and 5.

80 85

## Example 7

|                    | grammes |
|--------------------|---------|
| { Gum mastic       | 60      |
| { Linseed oil      | 30      |
| { Palm oil         | 30      |
| { Borax            | 20      |
| { Water            | 300     |
| { Casein           | 10      |
| { Water            | 100     |
| { Silicate of soda | 10      |
| { Water            | 500     |

Made up to final volume of two litres.

## Example 8

|                  | grammes |
|------------------|---------|
| { Gum mastic     | 30      |
| { Castor oil     | 30      |
| { Orange shellac | 20      |
| { Borax          | 40      |
| { Water          | 400     |
| Silicate of soda | 5       |

105

Made up to two litres.

## Example 9

|                  | grammes |
|------------------|---------|
| { Gum mastic     | 30      |
| { Castor oil     | 30      |
| { Japan wax      | 20      |
| { Borax          | 40      |
| { Water          | 400     |
| { Soda lye       | 6       |
| { Casein         | 26      |
| { Water          | 100     |
| Silicate of soda | 20      |

110 115

Made up to two litres.

I claim:

1. Process of treating vegetable and animal fibers, which consists in first treating the fibers in a sizing bath, comprising drying oils, casein, borax and water, of an oleatic emulsion free from sulphonated compounds using alkaline borates as dispersion agents with the addition of a soluble silicate; then passing the thus treated fibers through a deglutinating bath.

2. Process of treating vegetable and animal fibers, which consists in first treating the fibers in a sizing bath, comprising drying oils, casein, borax and water, of an oleatic emulsion free from sulphonated compounds using alkaline borates as dispersion agents with the addition of a soluble silicate; then passing the thus treated fibers through a deglutinating bath of low concentration for a short time.

3. Process of treating vegetable and animal fibers, which consists in first treating the fibers in a sizing bath, of an oleatic emulsion free from sulphonated compounds using alkaline borates as dispersion agents with the addition of a soluble silicate; then passing the thus treated fibers through a fixing bath of low concentration for a short time, said fixing bath comprising one of the group of compounds consisting of formates, acetates and sulphocyanides of calcium, zinc, aluminium and lead.

GEORGES LEFRANC.